# EUROPEAN PATENT SPECIFICATION

(11) **EP 3 667 218 B1**
(45) Date of publication and mention of the grant of the patent: **09.06.2021**
(21) Application number: 18211980.0
(22) Date of filing: 12.12.2018
(51) Int. Cl.: F26B 21/00, F26B 21/08

(54) **TIMBER DRYING PROCESS**
HOLZTROCKNUNGSVERFAHREN
PROCÉDÉ DE SÉCHAGE DU BOIS

(43) Date of publication of application: 17.06.2020
(73) Proprietor: Valutec AB, 931 27 Skellefteå (SE)
(72) Inventor: HÖGBLOM, Simon, 85640 Sundsvall (SE)
(74) Representative: Zacco Sweden AB

(56) References cited:
- WO-A1-2008/133583
- WO-A1-2013/158009
- WO-A1-2014/168559
- US-A- 4 255 870
- US-A1- 2008 184 589

## Description

### TECHNICAL FIELD

The present invention relates to a process for drying of timber comprising a heating step under conditions of moist heat and a subsequent drying step under conditions of dry heat. Further, the present invention relates to a unit adapted for carrying out the process.

### BACKGROUND ART

Drying is an important step in the processing of timber in a sawmill. In order to obtain a high-quality product it is important for carrying out the drying process under optimal conditions. Even in modern sawmills the timber drying process, however, is still associated with a substantial loss of energy. Approximately 80% of the added heating energy is lost, e.g. by venting out hot air to the ambient atmosphere without recovery.

WO 2014/168559 A1 describes a process for drying of timber in which an exhaust stream of moist hot air is removed from a chamber containing a first batch of timber and is passed into a chamber containing a following second batch of timber for heating said second batch of timber under conditions of moist heat.

US 2008/184589 A1 describes a drying process in which moist hot air recovered from an upstream process step is passed to a downstream process step.

Thus, it is an object of the invention to provide a more efficient use of energy in the timber drying process to save energy costs and to maintain high product quality.

### SUMMARY OF THE INVENTION

In general, the invention is based on the recirculation of moist hot air generated during a timber drying operation to pre-heat an incoming batch of timber. The invention relates both to the drying of timber in batch chamber driers and in continuous driers such as cross-circulating driers.

A first aspect of the invention relates to a process for drying of timber comprising the steps:
a) heating a first batch of timber in a chamber under conditions of moist heat, wherein a moist and heated first batch of timber is obtained,
b) drying the moist and heated first batch of timber in a chamber under conditions of dry heat, wherein a dry and heated first batch of timber is obtained,
wherein during drying step (b) an exhaust stream of moist hot air is removed from the chamber containing the first batch of timber and wherein at least a portion of said exhaust stream of moist hot air is passed into a chamber containing a second batch of timber for heating said second batch of timber under conditions of moist heat.

A second aspect of the invention relates to a unit for drying timber adapted for performing the process as described above. The unit comprises means for heating a batch of timber under conditions of moist heat for obtaining a moist and heated batch of timber and means for subsequently drying a moist and heated batch of timber under conditions of dry heat for obtaining a dry and heated batch of timber wherein the means for heating the timber under conditions of moist heat are at least partially provided by an exhaust stream of hot moist air generated during the drying of timber under conditions of dry heat.

In a particular embodiment, this aspect relates to a unit for drying timber comprising,
(a) a first chamber adapted for subjecting a first batch of timber to heating under conditions of moist heat and subsequent drying under conditions of dry heat,
(b) a second chamber adapted for subjecting a second batch of timber to heating under conditions of moist heat and subsequent drying under conditions of dry heat,
(c) means for passing an exhaust stream of moist hot air during drying the first batch of timber in the first chamber (a) into the second chamber (b) during heating the second batch of timber.

A further particular embodiment of this aspect relates to a unit for drying of timber comprising
a) a first chamber adapted for subjecting a batch of timber to heating under conditions of moist heat,
b) a second chamber adapted for subjecting said batch of timber to drying under conditions of dry heat,
c) means for passing said batch of timber after heating from the first chamber to the second chamber, and
d) means for passing an exhaust stream of hot moist air produced during drying the first batch of timber in the second chamber (b) into the first chamber (a) during heating a second batch of timber.

### DETAILED DESCRIPTION

The present invention relates to the drying of a batch of timber. The size of a timber batch used in the drying process may vary between different timber drying units depending on their size and capacity. In certain embodiments a batch of timber has a total volume of about 1 m³ to about 20 m³, e.g. about 5 m³ to about 16 m³ which may be formed from several packs, e.g. about 4 to about 50 packs of timber.

According to step (a) of the process, a first batch of timber is heated in a chamber under conditions of moist heat. In certain embodiments, this heating under conditions of moist heat is carried out until a dry temperature of about 40 °C to about 70°C and a wet temperature from about 40°C to about 70°C and the chamber is reached. The term "*conditions of moist heat*" indicates that there is a low difference between the dry temperature and the wet temperature in the chamber, particularly throughout the duration of step (a). In certain embodiments, the difference between dry temperature and wet temperature in the chamber during step (a) is about 25°C or less, about 20°C or less or about 15°C or less. Thus, the timber is heated under conditions of high absolute humidity. In particular, conditions of moist heat can be set by applying moist hot air to the timber in step (a) instead of just heat. This ensures that the timber is not substantially dried but only heated. Thus, in a preferred embodiment, moist hot air is fed into the chamber in step (a).

At the end of step (a) a moist and heated batch of timber is obtained. The amount of moisture is typically about 30 weight-% to about 180 weight-% water based on the total weight of the timber. Typically, the amount of moisture will be derived from the starting moisture content of the timber which may vary between different products and seasons. In particular embodiments, the moisture content of the timber does not substantially change during step (a), e.g. a change of 10 weight-% or less.

According to step (b) of the process, a moist and heated batch of timber is dried in a chamber under conditions of dry heat. The chamber can be the same as in step (a) or it can be a second chamber into which the timber is transferred after heating in step (a) is completed. The term "*conditions of dry heat*" indicates that there is a higher difference between the dry temperature and the wet temperature in the chamber, particularly at the end of step (b). In the beginning of step (b), the difference between dry temperature and wet temperature is small, preferably close to none, and then increases in the course of the procedure. In certain embodiments, step (b) comprises drying the timber under conditions of dry heat until a dry temperature from about 70°C to about 90°C and a wet temperature from about 40°C to about 70°C in the chamber is reached. The dry temperature in step (b) is preferably higher than the wet temperature in step (a). At the end of step (b), the difference between dry temperature and wet temperature may be about 10°C to about 35°C depending on the type of drier which is used. The amount of moisture in the timber after step (b) is about 6-20 weight-% or less based on the total weight of the timber after step (b).

The present invention is characterized in that during drying step (b) moist hot air is removed from the drying chamber and at least a portion of said moist hot air is recycled to heating step (a), particularly by passing an exhaust stream of moist hot air from a drying chamber containing a first batch of timber into a heating chamber containing a second batch of timber during the step of heating said second batch of timber under conditions of moist heat. Typically, the exhaust stream of moist hot air removed from the chamber in step (b) has a dry temperature from about 57°C to about 90°C, e.g. from about 60°C to about 85°C, and a wet temperature from about 57°C to about 75°C, e.g. from about 60°C to about 70°C. The difference between the dry temperature and the wet temperature in this exhaust stream is typically about 25°C or less or about 20°C or less and particularly about 5°C to about 20°C.

In a particular embodiment, the exhaust stream of moist hot air is passed into a heating chamber under conditions that a condensation of moisture from the exhaust stream takes place in the chamber, for example on the timber present in the chamber.

In a further particular embodiment, the exhaust stream of moist hot air is passed into a heating chamber without substantially reducing the moisture content thereof, e.g. without reducing the moisture content by about 20% or more and more particularly without reducing the moisture content thereof at all. Accordingly, essentially all humidity of the exhaust stream is reused for heating under conditions of moist heat in step (a). This can be achieved by supplying the exhaust stream as directly as possible and optionally in heat- insulated lines to process step (a) without passing through a heat exchanger in operation or other components in which substantial condensation of moisture can occur.

In a further particular embodiment, the exhaust stream of moist air is passed directly into the heating chamber, i.e. without first passing through a heat exchanger (or not through one in operation) such that the energy content of the exhaust stream of moist air is not substantially reduced. Essentially all heat energy and humidity of the exhaust stream are accordingly reused for heating in step (a).

In certain embodiments, no external steam is added to the exhaust stream of moist hot air before being passed into the chamber containing the second batch of timber. In other embodiments, external steam is added to the exhaust stream of moist hot air before being passed into the chamber containing the second batch of timber. External steam mainly needs to be added under conditions when the recycled steam is insufficient, for example, if multiple chambers need to be heated at the same time and/or when only few driers are in operation. Thus, according to the present invention the recycled exhaust stream of moist hot air from drying step (b) may constitute up to about 100% of the total air stream used for heating the second batch of timber.

In certain embodiments of the invention, additional water may be provided in the heating chamber when heating a batch of timber under conditions of moist heat, wherein the water may be added by spray nozzles or similar means. The additional water is provided into heating step (a) mainly under conditions where the difference between dry and wet temperature needs to be reduced in order to avoid a possible drying effect during heating step (a). Further, in certain embodiments additional heat may be introduced into the heating chamber when heating a batch of timber under conditions of moist heat, e.g. by means of a heater.

The process of the invention contributes to a significant reduction in the amount of externally added heat introduced into a heating chamber when heating a batch of timber under conditions of moist heat. In this context, the term "*externally added heat*" refers to the amount of heat which is externally generated and added to the process in contrast to the amount of heat which is provided by recycling of moist hot air according to the invention. For example the amount of externally added heat may be reduced by at least about 10%, 20%, 30%, 40%, 50%, 60%, 70%, 80% or 90% by introducing the exhaust stream of moist hot air from the heating of a previous batch of timber compared to the amount of externally added heat required for the heating step without recycling an exhaust stream of moist hot air. In particular embodiments, the process is operated without any external heat thereby reducing the external heat addition by up to about 100%.

The process of the present invention may be carried out in a batch chamber drier unit or into a continuous drier unit, e.g. a cross-circulating drier unit.

In a batch chamber drier unit heating step (a) and drying step (b) of a predetermined batch of timber are carried out in the same chamber. A typical sawmill may comprise a plurality of chambers each of which is adapted for performing heating step (a) and subsequently drying step (b). The drying process for predetermined batch of timber starts with insertion of a first timber batch into a first chamber. Then the newly inserted timber batch is heated under conditions of moist heat in the first chamber. During the heating it is important to have a low difference between wet and dry temperature as indicated above. After the batch of timber is sufficiently heated the actual drying process starts by introducing dry hot air into the first chamber until the timber has reached a desired moisture content.

According to the present invention an exhaust stream from a first chamber may be collected and passed into a different chamber in which heating of a further batch of timber is carried out. In particular embodiments, an exhaust stream from a plurality of chambers each containing a batch of timber is collected during drying step (b) and passed into at least one different chamber, particularly in a plurality of different chambers in which heating (a) of further batches of timber is carried out.

In this embodiment, the exhaust stream of moist hot air removed from the chamber in step (b) typically has a dry temperature from about 70°C to about 90°C and a wet temperature from about 50°C to about 70°C, e.g. a dry temperature of about 78°C and a wet temperature of about 60°C. The difference between dry temperature and wet temperature is typically about 20°C or less and more particularly about 5°C to about 20°C, e.g. about 18°C.

In a continuous drier, e.g. a continuous cross-circulating drier heating (a) of a predetermined batch of timber is carried out in a heating chamber and drying (b) of said predetermined batch is carried out in a drying chamber separate from the heating chamber. Thus, the batch of timber is transferred from a heating chamber to a separate drying chamber. A heating chamber may contain a plurality of individual heating zones and the batch of timber is passed through these individual zones during heating (a). Further, the drying chamber may contain a plurality of individual drying zones and the batch of timber is passed through individual zones during drying (b). In case the drying chamber contains a plurality of individual zones, the exhaust streams of moist hot air is preferably collected from zones wherein the first stages of drying (b) are carried out, i.e. wherein the timber still has a reasonably high moisture content.

In a continuous drier, the exhaust stream of moist hot air may be a stream of evacuation air originating from a single zone or a plurality of different zones in the chamber during step (b). The exhaust stream typically has a dry temperature from about 57°C to about 90°C and a wet temperature from about 45°C to about 70°C. The difference between the dry temperature and the wet temperature may be about 30°C or less, about 20°C or less, about 15°C or less or about 10°C or less and particularly about 5°C to about 10°C or less.

The second aspect of the invention relates to a unit for drying timber comprising means for heating timber under conditions of moist heat and subsequently drying the timber under conditions of dry heat, wherein the means for heating the timber under conditions of moist heat are at least partially provided by an exhaust stream of moist hot air generated during the drying of timber under conditions of dry heat.

In Figure 1, a batch chamber drying unit according to the state of the art is shown. The batch drier unit comprises a plurality of drier chambers KT 12-KT 21. Each chamber is operated separately except two shared air exits (10) comprising means, e.g. fans for supporting the removal of air from the drier chambers. The drying process in a first chamber starts with insertion of a timber batch into the chamber. The newly inserted batch of timber is heated in the chamber by introducing low pressure steam into the chamber. The low pressure steam is produced in a steam generator (12). The batch of timber is heated with steam under conditions of moist heat having a low difference between a wet temperature and dry temperature. When a batch of timber is sufficiently heated, the drying process starts by introducing dry hot air into the chamber until the timber has reached a desired moisture content. During the drying process the moist air from the chamber exits with the evacuation air at fan (10).

In Figure 2 a batch chamber drying unit according to the invention comprising drying chambers KT 12-KT 21 is shown. The unit is provided with pipes in each chamber, e.g. pipes (10a, 10b) for chamber KT 14. Pipes (10a, 10b) have openings and may provide inlet and/or outlet of air, as required. When air enters the pipe, air will exit the other pipe. Pipe (10a) works as an air exit when the chamber KT14 is operated in heating step (a). Both pipes (10a, 10b) may be provided with means, e.g. fans to obtain an active ventilation in the chamber, e.g. to support removal of air. Further a steam generator (12) is present. Instead of heating the timber exclusively with low pressure steam from the generator (12), however, the present invention provides means for heating the timber through recirculation of moist evacuation air from nearby chambers. For this purpose, evacuation air ducts (14) from each chamber are connected to provide a single stream of exhaust air for recycling back the evacuation air into another chamber. Valves (16) are installed in both evacuation air ducts (14) to direct the recirculated air into a specific chamber in which the timber is heated under conditions of moist heat. For this purpose, a ventilation pipe (18) is installed to lead the exhaust air stream from operating chambers into a specific chamber which shall be heated. For example, if chamber KT 14 is to be heated the respective valve (20) on pipe (10b) opens and the evacuation air from one or more surrounding chambers is passed into chamber KT 14 to heat the timber therein.

Measurement of the mean temperatures of the evacuation air from a drying chamber during the drying process gave a dry temperature of about 78°C and a wet temperature of about 60°C. These temperatures are maintained during the transfer of the evacuation air into a chamber in which timber is heated. When the moist evacuation air enters the chamber and contacts cool timber the moisture in the air condenses thereby providing a perfect heating climate. When using evacuation air from nearby chambers to heat the timber the heating energy is used more efficiently and cooler air with lower energy content will be evacuated out of the heated chamber by means of an exit, e.g. by exit (10) for chamber KT 14 into the atmosphere.

Figure 3 shows a continuous cross-circulating drying unit according to the state of the art with a single drying chamber (30). The drying chamber comprises a plurality of different drying zones (32a-32j). A batch of timber enters the drying chamber (30) through inlet (34) and is consecutively passed through the different drying zones during the drying operation.

The unit is operated without a separate heating chamber. The individual zones act as chamber driers with one heater and two evacuation vents in each zone. These evacuation vents provide inlet and/or outlet of air into the chamber, as required. During the drying step, the timber is moved from one zone to the next zone. The timber enters the unit at the first zone (32a) where the heating starts. The heating is conducted by a heater. Fresh water can be added in the heating zone to obtain a moist and warm climate. Thereafter, the timber is transferred to the next drying zone (32b), where the actual drying process starts. From there, the timber is further transferred to the subsequent drying zones (32c-32j).

A continuous drying unit according to the present invention is shown in Figure 4. It comprises an additional heating chamber (36) which may include a plurality of individual zones, e.g. three zones. The number of zones in the heating chamber (36) can vary. The heating chamber (36) is adapted for heating incoming timber under conditions of moist heat. It may be heated by evacuation air (38) from the drying chamber (30). For example, the evacuation air stream from drying zones 1-5 in (30) may be joined and transferred to heating chamber (36). Fans may be provided to direct the stream of warm and moist evacuation air (38). For example, fans may work in parallel to supply and remove air from the drying chamber (30) into the heating chamber (36). For example, the joint evacuating air flow (38) may have a dry temperature of 65°C and a wet temperature of 55°C. When the air flow (38) is introduced into heating chamber (36) and comes into contact with the timber the moisture in the air will condense. After condensation the dry temperature of the air may decrease to about 55°C-58°C while the wet temperature remains at 55°C.

In the heating chamber (36) heated water may be additionally introduced as a supplement to the evacuation air flow (38) in order to prevent drying and facilitating heating if the difference between dry and wet temperature is too high. Cool air with a low energy content leaves the heating chamber (36) via exit (40). Exit (10) may be provided as an active outlet supported by means, e.g. fans in order to facilitate the evacuation of air.

The invention enables a more efficient use of energy and decreases the drying time since the actual drying can start already in the first zone of drying chamber (32a).

## Claims

1. A process for drying of timber, comprising the steps;
a) heating a first batch of timber in a first chamber under conditions of moist heat, wherein a moist and heated first batch of timber is obtained,
b) drying the moist and heated first batch of timber in a second chamber under conditions of dry heat, wherein a dry and heated first batch of timber is obtained, wherein the chamber in step (b) can be the same or a different chamber than in step (a),
wherein step (a) preferably comprises introducing moist hot air into the chamber, wherein during drying step (b) an exhaust stream of moist hot air is removed from the second chamber containing the first batch of timber and wherein at least a portion of said exhaust stream of moist hot air is passed into the first chamber containing a second batch of timber for heating said second batch of timber under conditions of moist heat,
**characterized in that**
additional heat can be introduced into the first chamber containing the second batch of timber when heating the batch of timber under conditions of moist heat.

2. The process according to claim 1, wherein step (a) comprises heating the timber under conditions of moist heat until a dry temperature from about 40°C to about 70°C and a wet temperature from about 40°C to about 70 °C in the first chamber is reached, and wherein the difference between dry temperature and wet temperature in the first chamber during step (a) is about 25°C or less, about 20°C or less or about 15°C or less.

3. The process according to any of the claims 1 - 2, wherein step (b) comprises drying the timber under conditions of dry heat until a dry temperature from about 70°C to about 90°C and a wet temperature from about 40 °C to about 70 °C in the second chamber is reached, and wherein the difference between dry temperature and wet temperature at the end of step (b) is about 15°C to about 35°C.

4. The process according to any of the claims 1 - 3, wherein the exhaust stream of moist hot air removed from the second chamber in step (b) has a dry temperature from about 57°C to about 90°C and a wet temperature from about 57°C to about 75°C and wherein the difference between dry temperature and wet temperature is about 25°C or less or about 20°C or less and particularly about 5°C to about 20°C.

5. The process according to any of the claims 1 - 4, wherein upon passing the exhaust stream of moist hot air into the first chamber containing the second batch of timber, a condensation of moisture from the exhaust stream takes place in the first chamber containing the second batch of timber.

6. The process according to any of the claims 1 - 5, wherein the exhaust stream of moist hot air is passed into the first chamber containing the second batch of timber maintaining the moisture content of the exhaust stream to achieve condense heating in the first chamber containing the second batch of timber.

7. The process according to any of the claims 1 - 6, wherein external steam in an amount of up to about 8 MW of energy is added to the exhaust stream of moist hot air before being passed into the first chamber containing the second batch of timber.

8. The process according to any of the claims 1 - 7, wherein the amount of externally added heat introduced into the first chamber when heating a batch of timber under conditions of moist heat is reduced by at least about 10%, 20%, 30%, 40% or 50% and up to about 60%, 70%, 80% or 90% and preferably by up to about 100% by introducing the exhaust stream of moist hot air from the heating of a previous batch of timber.

9. The process according to any of the claims 1 - 8, wherein heating (a) and drying (b) of a predetermined batch of timber are carried out in the same chamber.

10. The process according to claim 9, wherein the exhaust stream of moist hot air removed from the second chamber in step (b) has a dry temperature from about 70°C to about 90°C and a wet temperature from about 55°C to about 70°C, e.g. a dry temperature of about 78°C and a wet temperature of about 60°C and wherein the difference between dry temperature and wet temperature is about 20°C or less and particularly about 5°C to about 20°C, e.g. about 18°C.

11. The process according to any of the claims 1 - 8, wherein heating (a) of a predetermined batch of timber is carried out in a heating chamber and drying (b) of said predetermined batch of timber is carried out in a drying chamber separate from the heating chamber.

12. The process according to any of the claims 1 - 11, wherein the exhaust stream of moist hot air removed from the second chamber in step (b) has a dry temperature from about 57°C to about 90°C and a wet temperature from about 45°C to about 70°C and wherein the difference between dry temperature and wet temperature is about 30°C or less, about 20°C or less or about 15°C or less or about 10°C or less and particularly about 5°C to about10°C.

13. A unit for drying timber comprising, means for heating timber under conditions of moist heat for obtaining moist and heated batch of timber, means for subsequently drying a moist and heated batch of timber under conditions of dry heat for obtaining a dry and heated batch of timber wherein, the means for heating the timber under conditions of moist heat are at least partially provided by an exhaust stream of hot moist air generated during the drying of timber under conditions of dry heat, **characterized in that** the means for heating timber under conditions of moist heating comprises a chamber, and which unit further comprising means for introducing additional heat into the chamber when heating the batch of timber under conditions of moist heating.

14. The unit according to claim 13 comprising,
(a) a first chamber adapted for subjecting a batch of timber to heating under conditions of moist heat and subsequent drying under conditions of dry heat,
(b) a second chamber adapted for subjecting a batch of timber to heating under conditions of moist heat and subsequent drying under conditions of dry heat,
(c) means for passing an exhaust stream of moist hot air during drying the first batch of timber in the first chamber (a) into the second chamber (b) during heating the second batch of timber.

15. The unit according to claim 13 comprising
(a) a first chamber adapted for subjecting a batch of timber to heating under conditions of moist heat,
(b) a second chamber adapted for subjecting said batch of timber to drying under conditions of dry heat,
(c) means for passing said batch of timber after heating from the first chamber to the second chamber, and
(d) means for passing an exhaust stream of hot moist air produced during drying the first batch of timber in the second chamber (b) into the first chamber (a) during heating a second batch of timber.

16. Use of a unit according to any one of claims 13-15 for the drying of timber, particularly in a process of any one of claims 1-12.

## Patentansprüche

1. Verfahren zur Holztrocknung, umfassend die Schritte;
a) Erwärmung eines ersten Holzbündels in einer ersten Kammer unter Bedingungen von feuchter Wärme, wobei ein feuchtes und erwärmtes erstes Holzbündel erzielt wird,
b) Trocknung des feuchten und erwärmten ersten Holzbündels in einer zweiten Kammer unter Bedingungen von trockener Wärme, wobei ein trockenes und erwärmtes erstes Holzbündel erzielt wird, wobei die Kammer in Schritt (b) dieselbe oder eine andere Kammer als in Schritt (a) sein kann,
wobei der Schritt (a) bevorzugt die Einführung von feuchter Warmluft in die Kammer umfasst, wobei während des Trocknungsschritts (b) ein Auslassstrom von feuchter Warmluft aus der zweiten das erste Holzbündel enthaltenden Kammer entfernt wird, und wobei mindestens ein Teil des Auslassstroms von feuchter Warmluft in die erste ein zweites Holzbündel enthaltende Kammer eingeleitet wird, um das zweite Holzbündel unter Bedingungen von feuchter Wärme zu erwärmen, **dadurch gekennzeichnet, dass**
bei Erwärmung des Holzbündels unter Bedingungen von feuchter Wärme eine Zusatzwärme in die erste das zweite Holzbündel enthaltende Kammer einführbar ist.

2. Verfahren nach Anspruch 1, wobei der Schritt (a) die Erwärmung des Holzes unter Bedingungen von feuchter Wärme umfasst, bis eine Trockentemperatur von etwa 40 °C bis etwa 70 °C und eine Nasstemperatur von etwa 40 °C bis etwa 70 °C in der ersten Kammer erzielt werden, und wobei der Unterschied zwischen der Trockentemperatur und der Nasstemperatur in der ersten Kammer während des Schritts (a) etwa 25 °C oder weniger, etwa 20 °C oder weniger oder etwa 15 °C oder weniger beträgt.

3. Verfahren nach einem der Ansprüche 1 bis 2, wobei der Schritt (b) die Trocknung des Holzes unter Bedingungen von trockener Wärme umfasst, bis ein Trockentemperatur von etwa 70 °C bis etwa 90 °C und eine Nasstemperatur von etwa 40 °C bis etwa 70 °C in der zweiten Kammer erzielt werden, und wobei der Unterschied zwischen der Trockentemperatur und der Nasstemperatur am Ende des Schritts (b) etwa 15 °C bis etwa 35 °C beträgt.

4. Verfahren nach einem der Ansprüche 1 bis 3, wobei der Auslassstrom von feuchter Warmluft, der in Schritt (b) aus der zweiten Kammer entfernt wird, eine Trockentemperatur von etwa 57 °C bis etwa 90 °C und eine Nasstemperatur von etwa 57 °C bis etwa 75 °C aufweist, und wobei der Unterschied zwischen der Trockentemperatur und der Nasstemperatur etwa 25 °C oder weniger oder etwa 20 °C oder weniger und insbesondere etwa 5 °C bis etwa 20 °C beträgt.

5. Verfahren nach einem der Ansprüche 1 bis 4, wobei bei Einleitung des Auslassstroms von feuchter Warmluft in die erste das zweite Holzbündel enthaltende Kammer eine Kondensation von Feuchte aus dem Auslassstrom in der ersten das zweite Holzbündel enthaltenden Kammer erfolgt.

6. Verfahren nach einem der Ansprüche 1 bis 5, wobei der Auslassstrom von feuchter Warmluft in die erste das zweite Holzbündel enthaltende Kammer eingeleitet wird, wobei der Feuchtegehalt des Auslassstroms zur Erzielung der Kondensationserwärmung in der ersten das zweite Holzbündel enthaltenden Kammer beibehalten wird.

7. Verfahren nach einem der Ansprüche 1 bis 6, wobei dem Auslassstrom von feuchter Warmluft ein externer Dampf in einer Menge von bis zu etwa 8 MW von Energie vor der Einleitung in die erste das zweite Holzbündel enthaltende Kammer zugesetzt wird.

8. Verfahren nach einem der Ansprüche 1 bis 7, wobei die Menge an extern zugesetzter Wärme, die bei der Erwärmung eines Holzbündels unter Bedingungen von feuchter Wärme in die erste Kammer eingeleitet wird, um mindestens etwa 10 %, 20 %, 30 %, 40 % oder 50 % und bis zu etwa 60 %, 70 %, 80 % oder 90 % und bevorzugt um bis zu etwa 100 % durch die Einführung des Auslassstroms von feuchter Warmluft aus der Erwärmung eines früheren Holzbündels verringert wird.

9. Verfahren nach einem der Ansprüche 1 bis 8, wobei die Erwärmung (a) und die Trocknung (b) eines vorgegebenen Holzbündels in derselben Kammer durchgeführt werden.

10. Verfahren nach Anspruch 9, wobei der Auslassstrom von feuchter Warmluft, der in Schritt (b) aus der zweiten Kammer entfernt wird, eine Trockentemperatur von etwa 70 °C bis etwa 90 °C und eine Nasstemperatur von etwa 55 °C bis etwa 70 °C, z.B. eine Trockentemperatur von etwa 78 °C und eine Nasstemperatur von etwa 60 °C, aufweist, und wobei der Unterschied zwischen der Trockentemperatur und der Nasstemperatur etwa 20 °C oder weniger und insbesondere etwa 5 °C bis etwa 20 °C, z.B. etwa 18 °C, beträgt.

11. Verfahren nach einem der Ansprüche 1 bis 8, wobei die Erwärmung (a) eines vorgegebenen Holzbündels in einer Erwärmungskammer durchgeführt wird, und die Trocknung (b) des vorgegebenen Holzbündels in einer von der Erwärmungskammer getrennten Trocknungskammer durchgeführt wird.

12. Verfahren nach einem der Ansprüche 1 bis 11, wobei der Auslassstrom von feuchter Warmluft, der in Schritt (b) aus der zweiten Kammer entfernt wird, eine Trockentemperatur von etwa 57 °C bis etwa 90 °C und eine Nasstemperatur von etwa 45 °C bis etwa 70 °C aufweist, und wobei der Unterschied zwischen der Trockentemperatur und der Nasstemperatur etwa 30 °C oder weniger, etwa 20 °C oder weniger oder etwa 15 °C oder weniger oder etwa 10 °C oder weniger und insbesondere etwa 5 °C bis etwa 10 °C beträgt.

13. Einheit zur Holztrocknung umfassend Mittel zur Erwärmung von Holz unter Bedingungen von feuchter Wärme zur Erzielung eines feuchten und erwärmten Holzbündels, Mittel zur anschließenden Trocknung eines feuchten und erwärmten Holzbündels unter Bedingungen von trockener Wärme zur Erzielung eines trockenen und erwärmten Holzbündels, wobei die Mittel zur Erwärmung des Holzes unter Bedingungen von feuchter Wärme zumindest teilweise durch einen Auslassstrom von feuchter Warmluft, die während der Holztrocknung unter Bedingungen von trockener Wärme erzeugt wird, vorgesehen sind, **dadurch gekennzeichnet, dass** die Mittel zur Erwärmung von Holz unter Bedingungen von feuchter Erwärmung eine Kammer umfasst, und welche Einheit bei Erwärmung des Holzbündels unter Bedingungen von feuchter Erwärmung ferner Mittel zur Einführung von Zusatzwärme in die Kammer umfasst.

14. Einheit nach Anspruch 13 umfassend
(a) eine erste Kammer, die dafür angepasst ist, ein Holzbündel einer Erwärmung unter Bedingungen von feuchter Wärme und einer anschließenden Trocknung unter Bedingungen von trockener Wärme zu unterwerfen,
(b) eine zweite Kammer, die dafür angepasst ist, ein Holzbündel einer Erwärmung unter Bedingungen von feuchter Wärme und einer anschließenden Trocknung unter Bedingungen von trockener Wärme zu unterwerfen,
(c) Mittel zur Einleitung eines Auslassstroms von feuchter Warmluft während der Trocknung des ersten Holzbündels in der ersten Kammer (a) in die zweite Kammer (b) während der Erwärmung des zweiten Holzbündels.

15. Einheit nach Anspruch 13 umfassend
(a) eine erste Kammer, die dafür angepasst ist, ein Holzbündel einer Erwärmung unter Bedingungen von feuchter Wärme zu unterwerfen,
(b) eine zweite Kammer, die dafür angepasst ist, das Holzbündel einer Trocknung unter Bedingungen von trockener Wärme zu unterwerfen,
(c) Mittel zur Einleitung des Holzbündels nach der Erwärmung von der ersten Kammer in die zweite Kammer und
(d) Mittel zur Einleitung eines Auslassstroms von feuchter während der Trocknung des ersten Holzbündels in der zweiten Kammer (b) erzeugter Warmluft in die erste Kammer (a) während der Erwärmung eines zweiten Holzbündels.

16. Verwendung einer Einheit nach einem der Ansprüche 13 bis 15 zur Holztrocknung, insbesondere in einem Verfahren nach einem der Ansprüche 1 bis 12.

## Revendications

1. Procédé de séchage de bois, comprenant les étapes consistant à ;
a) chauffer un premier lot de bois dans une première chambre dans des conditions de chaleur humide, un premier lot de bois humide et chauffé étant obtenu,
b) sécher le premier lot de bois humide et chauffé dans une deuxième chambre dans des conditions de chaleur sèche, un premier lot de bois sec et chauffé étant obtenu, la chambre à l'étape (b) pouvant être la même ou une chambre différente de celle à l'étape (a),
l'étape (a) comprenant de préférence l'introduction d'air chaud humide dans la chambre, pendant l'étape de séchage (b), un flux d'échappement d'air chaud humide étant retiré de la deuxième chambre contenant le premier lot de bois, et au moins une partie dudit flux d'échappement d'air chaud humide étant passée dans la première chambre contenant un deuxième lot de bois pour chauffer ledit deuxième lot de bois dans des conditions de chaleur humide, **caractérisé en ce que**
la chaleur supplémentaire peut être introduite dans la première chambre contenant le deuxième lot de bois lors du chauffage du lot de bois dans des conditions de chaleur humide.

2. Procédé selon la revendication 1, dans lequel l'étape (a) comprend le chauffage du bois dans des conditions de chaleur humide jusqu'à ce qu'une température sèche d'environ 40°C à environ 70°C et une température humide d'environ 40°C à environ 70°C dans la première chambre soient atteintes, et dans lequel la différence entre la température sèche et la température humide dans la première chambre pendant l'étape (a) est environ 25°C ou moins, environ 20°C ou moins ou environ 15°C ou moins.

3. Procédé selon l'une quelconque des revendications 1 à 2, dans lequel l'étape (b) comprend le séchage du bois dans des conditions de chaleur sèche jusqu'à ce qu'une température sèche d'environ 70°C à environ 90°C et une température humide d'environ 40°C à environ 70°C dans la deuxième chambre soient atteintes, et dans lequel la différence entre la température sèche et la température humide à la fin de l'étape (b) est d'environ 15°C à environ 35°C.

4. Procédé selon l'une quelconque des revendications 1 à 3, dans lequel le flux d'échappement d'air chaud humide retiré de la deuxième chambre à l'étape (b) a une température sèche d'environ 57°C à environ 90°C et une température humide d'environ 57°C à environ 75°C, et dans lequel la différence entre la température sèche et la température humide est environ 25°C ou moins ou environ 20°C ou moins et en particulier d'environ 5°C à environ 20°C.

5. Procédé selon l'une quelconque des revendications 1 à 4, dans lequel lors du passage du flux d'échappement d'air chaud humide dans la première chambre contenant le deuxième lot de bois, une condensation d'humidité provenant du flux d'échappement a lieu dans la première chambre contenant le deuxième lot de bois.

6. Procédé selon l'une quelconque des revendications 1 à 5, dans lequel le flux d'échappement d'air chaud humide est passé dans la première chambre contenant le deuxième lot de bois maintenant la teneur en humidité du flux d'échappement pour obtenir un chauffage par condensation dans la première chambre contenant le deuxième lot de bois.

7. Procédé selon l'une quelconque des revendications 1 à 6, dans lequel la vapeur externe dans une quantité allant jusqu'à environ 8 MW d'énergie est ajoutée au flux d'échappement d'air chaud humide avant d'être passée dans la première chambre contenant le deuxième lot de bois.

8. Procédé selon l'une quelconque des revendications 1 à 7, dans lequel la quantité de chaleur ajoutée extérieurement introduite dans la première chambre lors du chauffage d'un lot de bois dans des conditions de chaleur humide est réduite d'au moins environ 10%, 20%, 30%, 40% ou 50% et jusqu'à environ 60%, 70%, 80% ou 90% et de préférence jusqu'à environ 100% en introduisant le flux d'échappement d'air chaud humide provenant du chauffage d'un lot précédent de bois.

9. Procédé selon l'une quelconque des revendications 1 à 8, dans lequel le chauffage (a) et le séchage (b) d'un lot prédéterminé de bois sont effectués dans la même chambre.

10. Procédé selon la revendication 9, dans lequel le flux d'échappement d'air chaud humide retiré de la deuxième chambre à l'étape (b) a une température sèche d'environ 70°C à environ 90°C et une température humide d'environ 55°C à environ 70°C, par exemple une température sèche d'environ 78°C et une température humide d'environ 60°C, et dans lequel la différence entre la température sèche et la température humide est environ 20°C ou moins et en particulier d'environ 5°C à environ 20°C, par ex. environ 18°C.

11. Procédé selon l'une quelconque des revendications 1 à 8, dans lequel le chauffage (a) d'un lot prédéterminé de bois est effectué dans une chambre de chauffage, et le séchage (b) dudit lot prédéterminé de bois est effectué dans une chambre de séchage séparée de la chambre de chauffage.

12. Procédé selon l'une quelconque des revendications 1 à 11, dans lequel le flux d'échappement d'air chaud humide retiré de la deuxième chambre à l'étape (b) a une température sèche d'environ 57°C à environ 90°C et une température humide d'environ 45°C à environ 70°C, et dans lequel la différence entre la température sèche et la température humide est environ 30°C ou moins, environ 20°C ou moins ou environ 15°C ou moins ou environ 10°C ou moins et en particulier d'environ 5°C à environ 10°C.

13. Unité de séchage de bois, comprenant des moyens pour chauffer du bois dans des conditions de chaleur humide pour obtenir un lot de bois humide et chauffé et des moyens pour sécher ultérieurement un lot de bois humide et chauffé dans des conditions de chaleur sèche pour obtenir un lot de bois sec et chauffé, les moyens pour chauffer le bois dans des conditions de chaleur humide étant au moins partiellement fournis par un flux d'échappement d'air chaud et humide généré lors du séchage de bois dans des conditions de chaleur sèche, **caractérisée en ce que** le moyen pour chauffer le bois dans des conditions de chauffage humide comprend une chambre, et ladite unité comprend en outre des moyens pour introduire la chaleur supplémentaire dans la chambre lors du chauffage du lot de bois dans des conditions de chauffage humide.

14. Unité selon la revendication 13, comprenant
(a) une première chambre adaptée pour soumettre un lot de bois à un chauffage dans des conditions de chaleur humide et un séchage ultérieur dans des conditions de chaleur sèche,
(b) une deuxième chambre adaptée pour soumettre un lot de bois à un chauffage dans des conditions de chaleur humide et un séchage ultérieur dans des conditions de chaleur sèche,
(c) des moyens pour faire passer un flux d'échappement d'air chaud humide pendant le séchage du premier lot de bois dans la première chambre (a) dans la deuxième chambre (b) pendant le chauffage du deuxième lot de bois.

15. Unité selon la revendication 13, comprenant
(a) une première chambre adaptée pour soumettre un lot de bois à un chauffage dans des conditions de chaleur humide,
(b) une deuxième chambre adaptée pour soumettre ledit lot de bois à un séchage dans des conditions de chaleur sèche,
(c) des moyens pour faire passer ledit lot de bois après le chauffage de la première chambre à la deuxième chambre, et
(d) des moyens pour faire passer un flux d'échappement d'air chaud humide produit pendant le séchage du premier lot de bois dans la deuxième chambre (b) dans la première chambre (a) pendant le chauffage d'un deuxième lot de bois.

16. Utilisation d'une unité selon l'une quelconque des revendications 13 à 15 pour le séchage de bois, en particulier dans un procédé selon l'une quelconque des revendications 1 à 12.
